

May 4, 1937.

R. S. DEAN ET AL

2,078,933

PULVERIZING MINERAL AGGREGATES

Filed May 20, 1932.



Inventors

Reginald S. Dean and  
John Gross

By John J. McLaughlin, Attorney

## UNITED STATES PATENT OFFICE

2,078,933

## PULVERIZING MINERAL AGGREGATES

Reginald S. Dean, Washington, D. C., and John  
Gross, Minneapolis, Minn.

Application May 20, 1932, Serial No. 612,524

12 Claims. (Cl. 83—94)

Our invention relates in general to the treatment of inorganic materials, such as metallic ores. It relates more in particular to a method of and means for disintegrating such materials explosively by internal pressure.

Although our invention may be employed for the treatment of many types of naturally occurring inorganic materials, it has its greatest value in the crushing of ores preparatory to recovering the metals therefrom. It will be explained particularly therefore by comparison with present crushing processes as applied to ores.

Substantially all treatment of ores involves crushing of the ore to relatively fine size, the exact size depending upon the specific metal recovery process employed. Where flotation is used, for example, the particles must be of very small size; other methods of concentration may be carried on in which exceptionally fine grinding or disintegration is not necessary. Whatever the size of the particles, however, it has been customary heretofore to disintegrate the ore by externally applied pressure. One of the common methods, particularly where flotation is employed, is ball milling. This part of the process is not only very expensive, but has other disadvantages, particularly in the production of a relatively large amount of fines, and to the presence of fines can be traced much of the metal losses occurring during flotation. Another disadvantage of all methods of disintegration by external pressure is that there is always a great deal of useless work done in that the gangue or non-metalliferous portion of the ore is crushed as thoroughly as the metalliferous portion, thus representing a great loss of time and energy.

The principal object of our invention is to disintegrate ore in such a way as to avoid most of the objections to the present form of treatment.

Another object is the provision of an improved process for disintegrating ores by means of internal pressure.

Another object is the provision of a process which may be controlled to crush the ores differentially.

Another object is the preparation of ore in more satisfactory form for treatment by lixiviation than is accomplished by other methods of preparation.

Another object is the provision of a method for crushing ores which will effectuate a saving in time and labor and cheapen the overall cost of ore preparation.

Another object is the provision of an improved process adapted to produce a surface more amen-

able to flotation than can be produced by present processes.

Other objects and features of the invention may be apparent from a consideration of the following detailed description taken with the accompanying drawing, wherein a single figure illustrates novel apparatus with which the method may be practiced.

In accordance with the general features of the invention, the material to be treated is first given a preliminary crushing to reduce it to comminuted form. The sizes of the pieces produced in the preliminary step will be determined to some extent by the ore and the final treatment to be given the ore. In general, in this preliminary treatment, the pieces may be reduced to a size of from one-quarter to one-half inch. Any of the usual types of crushers, such as Symons' cone, for example, may be employed for this preliminary treatment.

Our invention utilizes the fact heretofore apparently little understood that ore material contains a relatively large amount of pores, small aggregates and fissures, which can be made to absorb liquid such as water, so that when subjected to a relatively high temperature and pressure in a closed container and suddenly discharged from the container, the sudden expansion of the water into steam will cause an explosive action and disrupt the ore. We have found that if the process is suitably controlled, as will be explained hereinafter, this explosive action can be utilized for the purpose of disintegrating the ore more satisfactorily and at a considerable saving over all present types of ore crushing. The process should be controlled to insure a full supply of water within the pores and interstices of the ore, including a control of the amount of water present with the ore but not confined within the pores thereof, as well as a proper control of the pressure and a proper control of the explosive treatment of the ore by the sudden release of the pressure.

All of these features have an important bearing upon the results secured, independently of the type of ore treated. The specific control, however, to secure the best results, is determined to some extent by the ore. It is also determined in part by the results desired. For example, if differential crushing is the desideratum, the control may be somewhat different than if differential crushing is not so highly important. In general, differential crushing occurs no matter how the process is practiced, but for particular ores modification of the pressure, for example, or the

amount of water present will have an effect upon the amount of differential crushing.

In order to insure a plentiful supply of water within the interstices of the ore, preliminary soaking of the ore material should be employed. The time of soaking will differ somewhat with different ores, and we have found that with some ores preliminary soaking for four or five days produces the best results. In most cases, soaking for a greater length of time does not improve the crushing action. The important point is to have the ore saturated with water and if the ore is of such a character that it is saturated in less time than four or five days, which is found to be the case with many ores, the soaking time may be decreased. Substances which lower the surface tension of water, including the common wetting agents such as soap, may be added to increase the penetration of the liquid into the interstices of the ore; such additions, however, are not necessary.

When the process is carried out by a plurality of explosions it is, of course, necessary to insure that water is introduced into the ore between the explosions. This is preferably accomplished by discharging the ore from an explosion into water. In this way, water is drawn into any interstitial spaces by the condensation of steam existing in them. As will be pointed out later, this discharge into water is advantageous from a standpoint of saving power.

The amount of water in addition to that introduced by soaking has an important bearing on the results. It affects the results not only from the standpoint of the amount of crushing obtained, but also has an effect upon the differential crushing action. We have found that with some ores, and with external heating, for the best results, the additional water present during the heating period, or what may be termed the added water, should be equal to at least half the weight of the ore, and even sometimes equal to the weight of the ore. The amount of water, however, is determined in part by the manner of heating, and also by the amount of differential crushing desired. In general, the amount should be kept as small as possible. When heating the container by external means, the amount of water is greater than when heating by means of high temperature steam, which is our preferred method. To secure the best results for differential crushing, all of the water except that necessary to fill the interstices is preferably drawn off before the ore is released to atmospheric pressure. The exact technique here also, however, is determined in part by the manner of heating.

We believe that the best crushing effect is obtained when the interstices of the ore are filled with a maximum amount of water at the time when the pressure is explosively released. When the container is heated by external means, all of the pressure within the container must be built up by evaporation of water in the container. An ample supply of water is, therefore, necessary to produce the requisite pressure and at the same time insure that there will be no drying out effect on the ore. Probably the pressure has the effect of still further saturating the ore with moisture and the presence of water equal to from one-half the weight to the total weight of the ore always maintains an ample supply of moisture for further saturation. Before explosion, however, the excess water is drawn off and most of the water present will be contained within the ore itself but not externally thereof. After draining the con-

tainer, the ore should not be allowed to stand as this might cause some drying out before the explosion.

When the ore is heated in the container by means of high pressure steam, no excess of water in the container is necessary. Ore, after soaking, is drained and introduced in this condition into the container. The presence of the high temperature saturated steam apparently accomplishes everything in the way of further saturating the ore during the heating period.

The ore for most purposes is exploded with only a relatively small amount of water present, except for that contained within the body thereof, and in many cases substantially no free water should be present for the best results. Draining off the excess water before explosion, effects a saving since most of the cost of practicing the process is determined by the amount of water converted into steam.

The pressure within the container at the time when the ore is discharged therefrom is preferably between 150 and 200 pounds per square inch. It is between these pressure ranges that the most favorable and most complete crushing action takes place. Below approximately 150 pounds, the amount of crushed material gradually decreases, while pressures greater than 200 pounds per square inch have very little increased effect on most ores. In certain types of ores, the crushing action decreases at pressures above 200 pounds per square inch and we have instances where the greatest crushing action takes place at about 150 pounds per square inch pressure and decreases slightly as the pressure is raised to 200 pounds per square inch. In certain types of ores, the greatest differential crushing action apparently takes place with pressures of about 120 pounds per square inch, but usually the amount of ore crushed at this pressure is decreased so that an advantage is obtained in sacrificing some differential crushing action in the interest of increased yield.

It should be borne in mind that the entire contents of the container should be in a state of equilibrium when the ore is discharged to atmosphere. This is best brought about by holding the final pressure for some considerable time before explosion. This promotes penetration of high pressure water into the interstices and assures that the temperature of such water is high and uniform throughout.

For convenience, the process will be further discussed by first considering an approved form of apparatus with which it may be practiced. Referring to the drawing, we provide a container 10 having a loading dome 11 closed by a revolvable valve 12, and an ore discharge chute 13 closed by a revolvable valve 14. The soaked ore is delivered by a suitable chute 16 to the valve 12. This valve, as shown, is so arranged as to close the chamber independently of its position so that the ore loaded into the valve, or feed chamber in which capacity it also acts, is delivered into the body of the container 10 by rotating the valve through 180°.

The valve 14 functions in a similar manner and constitutes the explosion chamber. The ore is continuously progressed through the container and delivered to the valve 14, which at time of delivery is in a reversed position to that shown. A quick rotation of the valve 14 discharges the ore contained in the valve and permits the entrapped water to be explosively converted into steam and crush the ore.

Within the container, we provide means for 75

continuously advancing the material therethrough. In the form shown, we provide a plurality of tiers 16, 17, 18 and 19, the bottom wall 21 of the container also functioning in the same manner as the tiers. A vertical shaft 22 carries a series of paddles or agitators 23 which pass over the ore supporting tiers and gradually move the ore from an upper tier to the next lower tier. The tiers are provided with ore discharge positions alternately at the outside edge and at the inner edge in the manner shown. For example, the ore is discharged from the outside edge of tier 16 to the outside edge of tier 17, whence it is gradually moved to the inside edge of tier 17 and discharged to the inside edge of tier 18. In the case of the lowermost tier 21, this coincides in a horizontal plane with the entrance to the discharge chute 13, so that the ore delivered from this tier drops into the valve 14.

The shaft 22 is suitably journaled and slowly rotated by means of a pair of beveled gears 24 and 26, the driving beveled gear 26 being connected to a shaft 27, journaled through the side walls of the container and packed to prevent loss of pressure.

Steam is continuously admitted through a steam pipe 28 to the interior of the container for heating the ore and maintaining the requisite pressure on the ore and in the interstices thereof. The movement of the ore downwardly on the tiers is timed so that an equilibrium condition exists in the ore when it is delivered to the valve 14. The quick rotation of the valve 14 disturbs its equilibrium condition and causes the crushing.

The ore delivered into the feed chamber is wet, having been previously saturated with water by soaking a suitable length of time. The excess water, however, has been drained off, care being taken to avoid a drying out of the ore, however, before it is delivered to the feed chamber. Saturated steam is employed for heating and this may be depended upon to provide an ample supply of water for the explosive action.

There are several factors which have an effect upon the shattering process. They may be listed in general as follows:

- (a) Explosion of water in the structure of the mineral;
- (b) Explosion of water in pores or cracks;
- (c) Shattering by impact of particles on each other and against the walls of the explosion chamber or against the walls of a receiving bin;
- (d) Shattering by unequal heating due to evaporation of water producing sudden cooling of surface.

Our process is preferably governed by a control of the factors hereinabove discussed so that the process involves crushing only by means of (a) and (b), or at least principally by (a) and (b). This gives the greatest amount of differential crushing. We have found that if there is a large amount of water present, a great deal of the explosive action is due to the shattering of particles on each other, as described in (c). Possibly some of this effect, when a large amount of water is used, is also due to concussion or force entirely applied from without through a layer of water against the side walls of the particles. This factor is best explained by comparison to the depth bomb method employed against submarines, in which the water itself being non-compressible acts as a ram. This would be expected to have the effect of partially decreasing the amount of crushing action if an exceedingly large amount of water were employed, and also of

crushing the gangue as much as the mineral content of the ore. Experiments have shown that this seems to be the case, as where a large amount of water is used, the amount of crushing was decreased and there was substantially no differential crushing action. 5

Not only is the differential crushing action increased by employing a small amount of water, but the cost of the process is also greatly decreased. It is obvious that the cost is principally determined by the amount of water evaporated. Preferably we employ counter-current circulation of boiler feed water in a way to further increase the economy; theoretical calculation shows that the process can be carried on so that the 15 actual energy input will amount to only about 1000 B. t. u.'s per ton of ore treated. By employing the crushed ore to preheat the boiler feed water and heating the ore with saturated steam, the process can be carried on continuously with apparatus of the character described so that almost all heat energy consumed is in the actual crushing.

When the ore is to be re-explored, it is of considerable value, particularly when a continuous 25 process is employed, to discharge the ore so that immediately after the explosion it is precipitated into water, thus facilitating the refilling of the pores while the ore is still somewhat warm, and also heating the water which can be circulated 30 to the boiler feed pump or injector.

Although we prefer to heat the ore with saturated steam, our process may be carried out by the application of external heat to the container. This manner of carrying out the process is not 35 so desirable from some standpoints, however, because there will be some drying out of the ore near the outside of the container where the heat is introduced. For example, to maintain a steam pressure of 150 pounds per square inch above the ore bed, the lower part of the ore will be heated to a temperature above that at which the water and steam are in equilibrium at this pressure, and some water will be distilled from the ore close to the point at which the heat is applied. 40 When heating is accomplished by means of saturated steam, however, this difficulty is obviated. 45

One of the advantages of practicing our process in the manner described resides in the substantial elimination of slime production in the 50 soft ores such as iron ores. This is due to eliminating crushing to a great extent by means of impact, as referred to under (c) and (d) above. Another feature and advantage is that the ore prepared is more susceptible to flotation partly 55 on account of the lack of slimes below a critical size and partly due to the fact that the surface resulting from the crushing appears to be more amenable to flotation.

Another advantage resulting from the practice of our process in the manner described resides in the production of a large amount of free surface of valuable material which may be included in a large amount of worthless material. This is true because the contact between two different kinds of minerals is usually susceptible to penetration by water so that in the explosion process the breaks most frequently take place at the surface of the included minerals. This large amount of exposed surface is particularly 60 valuable when it is desired to remove the mineral by lixiviation. 65

When a large production of small size ore particles is desired, as for example for flotation purposes, it is preferable to re-explode the ore in 70 75

a continuous series of operations. This is accomplished by screening or any suitable means for separating the ore according to size. The separation may be carried out in such a way that 5 the gangue constituents can be largely eliminated. Due to the differential crushing action which we obtain, all particles over a certain size (the exact size depending upon the ore) will be found to contain very little mineral matter and 10 can be separated out before reintroducing the uncrushed ore bearing particles to the explosion crushing treatment.

In connection with the above, it is found that a valuable mineral will be crushed more easily 15 than the worthless gangue. Occasionally, however, this is not the case, and sometimes the behavior is just the reverse and the gangue will be shattered more readily, leaving the valuable ore in the form of hard particles. Separation under 20 the latter conditions will then be on the basis of the larger particles containing the valuable ore, and any of the usual methods of separation, classification, sizing or the like can be used. The ore may then be re-explored, or further treated 25 in any suitable manner. There may be times, however, in which it will be desirable to re-explode the entire ore body without intermediate screening.

What we claim as new and desire to protect by 30 Letters Patent of the United States is:

1. The method of pulverizing mineral substances and aggregates which comprises soaking the mineral substance in water, draining the excess water therefrom, introducing the water 35 soaked mineral substance into a closed container, admitting saturated steam into the container to heat the mineral substance, and discharging the mineral substance from the container whereby the water therein is explosively converted into 40 steam and disrupts the substance.

2. The method of pulverizing mineral substances and aggregates which comprises soaking the mineral substances in water, introducing the water soaked mineral substance into the container, introducing saturated steam into the container, continuously progressing the material 45 through the container and counter to the circulation of the steam, whereby the mineral substance is raised to substantially the temperature 50 of the steam as it passes through the container, and continuously discharging a portion of the hot mineral substance from the container whereby the water therein is explosively converted into vapor and disrupts the material.

55 3. A method of pulverizing mineral substances and aggregates which comprises heating the mineral substance with water in a closed container by means of steam introduced therein until an equilibrium condition exists in which a high 60 steam pressure is above the mineral substance and its pores are filled with water, controlling the amount of water so that substantially all of the water present is contained in the pores of the mineral substance, and successively releasing 65 amounts of the mineral substance to atmospheric pressure.

4. The method of pulverizing mineral substances and aggregates which comprises heating the mineral substance in the presence of water in 70 a closed container until a relatively high vapor pressure is developed therein, the amount of water being controlled so that substantially all that is present is contained in the pores and interstices of said mineral substances, discharging 75 the mineral substance from the container where-

by the liquid is explosively converted into vapor and the mineral substance pulverized, discharging the crushed ore immediately into water to cause the pores thereof to take up additional water, recharging the ore and water into the container, and again treating the ore to cause an explosive crushing thereof.

5. The method of pulverizing mineral substances and aggregates which comprises preliminarily processing the substances to produce 10 aggregates of substantially uniform size, suitable for crushing, soaking said substances in water, charging the water soaked substances into a sealed container, the amount of water being so controlled that substantially all that is present 15 is contained in the pores and interstices of said mineral substances, applying heat to said container by admitting saturated steam thereinto until a relatively high temperature and a pressure between 150 pounds and 200 pounds per 20 square inch are developed therein and an equilibrium condition established between vaporized and unvaporized water, and suddenly opening the container to discharge the substances therefrom.

6. The method of pulverizing mineral substances and aggregates which comprises preliminarily processing the substances to produce aggregates of substantially uniform size, suitable for crushing, soaking said substances in water, charging the water soaked substances into 30 a sealed container, applying heat to said container by admitting saturated steam thereinto until a relatively high temperature and pressure are developed therein and an equilibrium 35 condition established between vaporized and unvaporized water; draining the free water from said substance, and suddenly opening the container to discharge the substances therefrom.

7. In a continuous process of pulverizing mineral substances and aggregates, the steps comprising, soaking the substance in water, successively introducing portions of the water soaked substance into a container, continuously progressing the material thru said container and heating the same to raise the temperature thereof as 4 it passes thru said container and to build up a high pressure in said container, and successively discharging amounts of the heated substance from said container into water whereby the water contained in said material is explosively 5 converted into vapor, disrupting the substance and simultaneously preheating said water to condition the same for use in said continuous process.

8. In a continuous process of pulverizing mineral substances, the steps comprising, soaking 5 the substance in water, successively introducing amounts thereof into a container, introducing saturated steam into the container at a pressure between about 150 and 200 pounds per square inch, continuously progressing the material thru 6 said container and heating the same to raise the temperature thereof as it passes thru said container, and successively discharging amounts of the heated substance from said container into water.

9. In a continuous process of pulverizing mineral substances, the steps comprising, soaking the substance in water, successively introducing amounts thereof into a container, introducing saturated steam into the container at a pressure 7 between about 150 and 200 pounds per square inch, continuously progressing the material thru said container and heating the same to raise the temperature thereof as it passes thru said container, and successively discharging amounts 7

of the heated substance from said container into water whereby the water contained in said material is explosively converted into vapor, disrupting the substance and simultaneously preheating 5 said water to condition the same for use in said continuous process.

10. The method of effecting a differential pulverization of ore comprising ore mineral and associated gangue material which comprises soaking the ore in subdivided form in an aqueous medium to effect substantial saturation of said ore with water, placing the saturated ore into a chamber, closing said chamber and then introducing thereinto steam to build up the temperature and the 15 pressure in said chamber to a relatively elevated extent, and then suddenly releasing said pressure whereby the ore mineral is disrupted while the gangue material associated therewith is relatively unaffected whereby separation of the ore 20 mineral from the gangue material is facilitated.

11. The method of effecting a differential pulverization of ore comprising ore mineral and associated gangue material, said ore being in the form of aggregates of substantially uniform size, 25 suitable for crushing, comprising preliminarily soaking said ore in an aqueous medium to effect a substantial saturation thereof with water, pass-

ing steam into contact with said ore while disposed in a closed chamber whereby the ore is heated to an elevated temperature and a relatively high pressure is built up in said chamber, and then suddenly opening the chamber to release the pressure therein whereby the ore mineral is disrupted while the gangue material associated therewith is relatively unaffected whereby separation of the ore mineral from the gangue material is facilitated.

10. The process of pulverizing mineral substances which comprises soaking the substances in water, draining off excess water to leave a pre-determined amount of water in said substances, subjecting said pretreated substances, containing 15 substantially only that amount of water which is retained in the pores and interstices of said substances, in a closed container, to direct contact with saturated steam at a relatively high temperature and pressure until an equilibrium is 20 established between vaporized and unvaporized water, and then suddenly opening the container to permit sudden expansion of the superheated water whereby pulverization of the mineral substances is effected.

REGINALD S. DEAN.  
JOHN GROSS.